

Nov. 17, 1942.

M. SKOLNIK

2,302,270

## PULP MAKING PROCESS

Filed April 12, 1938

4 Sheets-Sheet 1



INVENTOR  
*Max Skolnik*  
BY *Evans & McCoy*  
ATTORNEYS

Nov. 17, 1942.

M. SKOLNIK

2,302,270

PULP MAKING PROCESS

Filed April 12, 1938

4 Sheets-Sheet 2



Fig. 2



Fig. 4

INVENTOR  
*Max Skolnik*  
BY  
*Evans & McCoy*  
ATTORNEYS

Nov. 17, 1942.

M. SKOLNIK

2,302,270

## PULP MAKING PROCESS

Filed April 12, 1938

4 Sheets-Sheet 3



INVENTOR  
*Max Skolnik*  
BY  
*Evans & McCoy*  
ATTORNEYS

Nov. 17, 1942.

M. SKOLNIK

2,302,270

PULP MAKING PROCESS

Filed April 12, 1938

4 Sheets-Sheet 4



INVENTOR  
*Max Skolnik*  
BY  
*Evans & McCoy*  
ATTORNEYS

## UNITED STATES PATENT OFFICE

2,302,270

## PULP MAKING PROCESS

Max Skolnik, Chicago, Ill.

Application April 12, 1938, Serial No. 201,525

8 Claims. (Cl. 92—13)

This invention relates to the manufacture of pulp from fibrous, vegetable material, such as cereal straws, grasses, cornstalks, bagasse, and the like.

An object of the invention is to provide an improved method for treating fibrous, vegetable materials, such as straw and the like, in the manufacture of paper pulp therefrom.

Another object of the invention is to provide an economical method of producing a high grade of paper pulp from straw and the like, and which method may be carried out easily.

A further object of the invention is to provide a continuous method of making pulp from straw and the like, in which means are provided to regulate the strength of the cooking liquor within predetermined limits.

Another object of the invention is to provide an easy and flexible control of the cooking of the fibrous, vegetable material by regulating the time of cooking and by regulating the temperature of the cooking liquor, as well as regulating its strength.

Still another object of the invention is to provide a method and apparatus in which the soluble products obtained from cooking the straw may be recovered and the free alkali content reused in the cooking process.

A further object is to provide a method of cooking fibrous, vegetable material which may be readily varied for given fibrous, vegetable materials to produce pulps having widely varying characteristics and suitable for many useful applications.

In the drawings is diagrammatically illustrated an embodiment of this invention which is adapted for carrying out the method, and which forms a complete plant for the production of pulp from raw material and the recovery of soda and lignins. The invention is illustrated in connection with straw from wheat or the like and, for convenience, the term "straw" will be used in the specification, but it is to be understood that other types of fibrous, vegetable material, such as grasses, stalks, vines, etc., may be treated according to the method and with the apparatus disclosed herein.

In the drawings,

Figure 1 is a side elevational view, somewhat diagrammatic, of apparatus in accordance with this invention, and adapted for carrying out the method of this invention.

Fig. 2 is an enlarged sectional view of the cooking tank taken on line 2—2 of Fig. 1.

Fig. 3 is an end view of one of the cooking baskets.

Fig. 4 is a side view of a modified form of cooking basket.

5 Fig. 5 is a side elevation, largely diagrammatic, of apparatus to reduce the solid material or straw, after it has been cooked, to a pulp suitable for paper or the like.

10 Fig. 6 is a side elevation, largely diagrammatic, of the recovery apparatus for the recovery of the free alkali content and lignins from the liquor in which the straw has been cooked.

15 Bales 1 of straw, with their ties cut and removed, are moved along conveyor 2 to a revolving, perforated screen or drum 3 which serves as a chaff screen and permits loose chaff and dirt to drop therefrom. The loosened straw coming from the drum is carried by conveyor 4 to suitable cutters 5, from which it passes into the opening 6 of a pneumatic conveyor 7. Above the cutters a suitable arrangement of dust collectors 8 may be disposed if, desired, to remove dust as the straw is cut.

20 The pneumatic conveyor 7 carries the loosened, cut straw to a suitable type of separator for further separating the dust and dirt. Preferably, such a type of separator is a cyclone separator, as indicated at 9, and is provided with a suitable fan 10 and exhaust outlet. The loose straw, from 25 which the dust and fine material have been separated, passes through the discharge end of the separator 9 to a suitable trough or container 11. This container is provided with a conveyor 12 to move the straw longitudinally thereof, and such 30 a conveyor is preferably one of the screw type and gear driven by suitable motor 13, so that it may be readily stopped and started.

35 Into the top portion of the container 11 is projected a wetting and wilting medium for wilting the straw before charging it into baskets or containers for cooking. The straw may be wilted with steam or sprayed with hot water, fresh hot cooking liquor, black liquor from the process, or a combination of these. In the drawings is 40 shown a suitable spray 14, which is preferably supplied with hot cooking liquor.

45 After the straw has been wetted and wilted it is compacted by causing it to pass through a duct of smaller size than the wilting trough. This may be conveniently done by providing a tapered duct 15 adjacent the trough 11. This tapered duct 15 may also be provided with a further wilting means, such as the ring pipe 17 and connections 18 to conduct steam into the duct 15 to the straw, and thereby further the wilting and com-

pacting of the straw in this portion of the apparatus.

After the wilted straw has been compacted it passes on to the discharge box 19. This box is disposed above a cooking basket, to be later described, and is provided at the bottom with a suitable discharge gate, which may take the form of a double clam gate 20, as indicated. The purpose of the gate is to withhold in the box the material discharged into it during the time of exchange of an empty basket for a loaded one.

The discharge box 19 is preferably of a size such that it holds somewhat more than the contents of a cooking basket 21, so that the operation of the wilting and compressing apparatus may be continuous, rather than interrupted after the filling of each basket. Also, the discharge box is preferably made so that it increases in cross sectional dimension in a downward direction. This may be by having two or more of the sides taper outwardly. The purpose of this increase in area from the inlet portion of the discharge box to the outlet portion thereof is to facilitate descent of the wilted straw material through the box. If desired, however, a suitable ram may be disposed above the discharge box 19 to pack the straw in the cooking basket 21, which is disposed below the box 19. Such a ram should have a stroke of sufficient length so that on its return it would come out of the box 19 and not hinder the discharge of wilted straw from the duct 15.

The wilted and compacted straw is discharged from the bottom of the box 19 successively into foraminous or fenestrate containers or baskets, one of which in its loading position is indicated at 21<sup>a</sup>. There are a plurality of such baskets of the same size. They may be formed of heavy wire mesh or perforated sheet metal suitably reinforced, and fitted with covers which may be readily opened at one or both ends. The baskets 21 are supported by attached trunnion rollers or wheels 22, adapted to permit easy travel of the baskets along horizontal or inclined tracks, and are further fitted with lugs or projections, so that when progressing along such tracks, in the manner described, there may be a definite space between the faces of each basket and those of the adjacent baskets.

After a basket 21 is filled with straw from the discharge box it is moved along the track 23 to track 24, where the basket enters a hood or enclosure 25, disposed above the cooking tank 26. The baskets progress along the track 24 of the hood until they are received by the cage 27 of a suitable hoist or elevator 28.

The baskets may be of any desired shape, a suitable shape being that shown in the drawings (see Figs. 2 and 4), in which the baskets are shown substantially rectangular in cross section and having substantially rectangular faces. If desired, two opposite sides or faces of the basket may be tapered, or all four of the sides or faces may be tapered, thereby causing the cross sectional area of the basket to increase longitudinally, and thus facilitate discharge of the contents. Side and end views of the basket are shown in Figs. 2 and 3, and it will be noted that reinforcing members, such as channels 29, may be disposed along the sides of the basket substantially at the middle portion thereof to receive the thrust of the ram 30 and to transmit such thrust to other baskets in the course of travel through the cooking tank. Also, these members act as spacers to provide sufficient space between

the baskets as they progress through the cooking tank to allow adequate circulation of the cooking liquor between the baskets and through the foraminous faces thereof.

Disposed across the end portions of the baskets 5 are suitable reinforcing members 31 connecting the reinforcing members 29, and which act as supports for suitable wheels or rollers 22, which may be mounted on axles 32 supported by plates 33 carried by members 34. The rollers or wheels 22 may ride on suitable tracks, such as the angle iron tracks 35, carried on the inside of the tank, whereby the baskets are easily propelled through the cooking tank.

10 In Fig. 4 is shown a modified form of basket. In this form of basket the bottom portion is formed with reentrant V portions 36 which facilitates the penetration of the cooking liquor through the contents of the basket, even though the contents be quite dense and compacted.

15 The cage of the hoist mechanism is provided with suitable means to engage the trunnions of the basket and hold the basket against displacement relative thereto, so that it may be lowered into the cooking tank.

20 After a basket of straw has been deposited in the cooking tank by the elevator 28 it may be moved horizontally along the tank by means of a suitable ram 30. Movement of the ram to push the last basket one basket space along the cooking tank moves all the baskets in the cooking tank the same amount. It is, of course, desirable that the pusher or piston rod of the ram enter the tank through a suitable stuffing box, and it is preferably provided within the tank with a shoe extending laterally across the face of the basket.

25 The cooking tank 26 is preferably substantially rectangular in cross section and made of any suitable construction, such as steel plate, suitably stiffened, but with the bottom somewhat inclined toward the outlet 37 to facilitate cleaning. Along the sides of the cooking tank are tracks 35 upon which the trunnions of the baskets travel, the baskets being impelled progressively through the tank by the thrust of the ram 30.

30 When a basket reaches the end 38 of the cooking tank it is in position to be raised by a suitable hoist elevator 39, which is similar in construction to the elevator 28 where the baskets are introduced. A ram 40 is also provided in order to propel the elevated basket laterally until the trunnions engage the tracks 41 disposed above the cooking tank.

35 Upon return of the ram 40 to its withdrawn position another basket may be lifted from the cooking tank by the hoist 39. As the baskets progress along the track 41 above the cooking tank, the cooking liquor drains therefrom into the pan or hopper 42, from which the drainings may be returned directly to the cooking tank by means of the pipe 43.

40 Adjacent the pan 42 another pan 44 is disposed in the path of the baskets as they progress along the track 41. Suitable spray or shower pipes 45 disposed above the baskets 22 are arranged to shower on the cooked straw in the baskets a liquid which is preferably weak black liquor obtained by pressure extraction in a successive stage of the process, but which may be weak wash liquor, or even fresh water. By such spraying, more of the entrained cooking liquor and lignins are removed from the cooked or reduced straw.

45 It is preferred to employ a weak black liquor for this purpose, as thereby the weak liquor is

strengthened and rendered more suitable for economical recovery of the alkalies and lignins contained in the liquor. The pipe 46 from this pan leads to the recovery system.

The sprays may extend over any desired number of baskets, there being a number of stations, however, between the last spray and the end of the track 41, so that the baskets may drain for a suitable period of time. Upon leaving the track 41 the basket is dumped to discharge the contents thereof onto a suitable conveyor 47. Any suitable mechanism for this purpose may be employed to so discharge the contents and to dispose the basket in upright position to roll on the tracks 23, where it may receive another load of straw to be cooked. Diagrammatically indicated in the drawings is a revolving cage 48 which inverts the basket to discharge the contents on the conveyor 47 and returns the basket to upright position for reception on the track 23, where it may receive straw to be cooked.

The cooking or steeping liquor is preferably a dilute solution of sodium hydroxide. The concentration of the cooking liquor, its temperature, and the time of cooking, depend upon the particular type of straw or fibrous vegetable matter being treated, and also upon the desired amount of softening or loosening of the bonding material holding the cellulose fibers together.

For a straw such as the straw of wheat, oats or rye, a 1% to 2% solution of sodium hydroxide is very desirable for the cooking liquor. The temperature of the cooking liquor is somewhat dependent upon the concentration of the sodium hydroxide, i. e., with higher percentages of sodium hydroxide the temperature need not be so high. It is to be noted, however, that the percentage of sodium hydroxide for cooking straw, such as wheat straw, should not be above 5% or 6%. It is not necessary to use high percentages of sodium hydroxide in my process because the cooking bath is preferably maintained at a substantially constant causticity. When the concentration of sodium hydroxide is too high it is likely to give the material too drastic a cook for many purposes. With a 1% to 2% concentration of sodium hydroxide, and with the straws above mentioned, a temperature between 175° F. and the boiling point is satisfactory.

The time that the straw passes through the cooking tank is also dependent upon the type of pulp that is being produced and the particular raw material. Where it is not desired to give the straw too drastic a cook, it has been found that when the straw is immersed in the cooking solution for a period of thirty minutes to one hour, with a sodium hydroxide solution of 1% to 2% and a temperature around 200° F., very desirable results are obtained.

By means about to be described it will be seen that the cooking liquor is constantly reheated and revivified, and may be automatically kept to any desired temperature. Also, the time of cooking may be varied by varying the length of time during which the baskets are kept in the cooking tank, so that the process is readily adaptable for a large variety of types of fibrous vegetable material, and the process and apparatus may be operated to cook such material very efficiently to the desired degree, depending upon the results to be obtained, that is, whether it be desired to disintegrate the material rapidly or to a great degree in the cooking tank, or whether it be desired to cook the material a minimum amount to loosen the encrusting and intercellular constituents of the raw material, so that they may be

readily separated from the fibers by subsequent treatment, and the fibers retain a maximum strength and length.

While a rough, coarse and stiff pulp may be obtained in a relatively short cooking time, and with a relatively low strength cooking liquor, and cooking at a relatively low temperature, increasing the causticity of the cooking liquor, increasing the temperature thereof, and increasing the time of cooking, will materially change the characteristics of the pulp, so that it is reduced to a point where it may be bleached to form white paper. Between these ranges pulp may be obtained which is suitable for egg crates, container board, corrugated board, and many other purposes.

In order to control the strength and causticity of the cooking liquor, and also the temperature, liquor is withdrawn from the tank outlet by pipe 50, from which it is pumped by pump 51 through pipes 52, 53 to the heater 54, supplied with steam through pipe 55. Into the pipe 50 connects pipe 56, having a valve 57 by which fresh caustic liquor may be introduced into the system.

From the heater the hot liquor is transported through pipes 58, 59 to a suitable header pipe 60, which preferably has a plurality of connections through which liquor is distributed to the cooking tank. The header pipe may be disposed above the cooking tank and discharged down into it, but it is to be understood that return of the hot liquor may be made into the sides or bottom portions of the cooking tank, if desired. A pipe 58a is connected by a suitable valve to the outlet pipe 58 of the heater, and hot cooking liquor may, if desired, be carried through pipe 58a to pipe 14a. Pipe 58a may be connected to pipe 14a for supplying hot cooking liquor for the spray 14. Spray 14, however, may be supplied with steam or other hot liquid for wilting purposes.

Inserted into a fitting in the pipe 59 is shown the stem or actuating element of thermostat valve 61 in the steam supply pipe, by means of which the temperature of the cooking liquor may be maintained substantially constant at any desired point.

Also connected to the tank outlet pipe 50 is a pipe 62 with valve 63. This pipe can be used to drain the cooking liquor from the tank when operation is to be interrupted or stopped, but primarily this pipe may be employed to control the causticity of the cooking liquor, as will be explained.

Due to action of carbon dioxide in the air and in gases given off by the straw or vegetable fibrous material under action of the cooking liquor, a conversion of caustic soda into sodium carbonate takes place in the cooking tank, which, without withdrawal of a portion of the liquor, may result in so great a conversion of caustic soda as to affect the proper operation of the cooking process. By withdrawal of a portion of the liquor through pipe 62, regulated by valve 63, and replacement of the withdrawn volume by fresh cooking liquor through the pipe 56, the accumulation of sodium carbonate in the cooking liquor may be held within any desired limit. The withdrawn liquor may be conveyed to the recovery system, wherein it is concentrated, the lignins separated, and the alkaline liquor recausticized.

A conveyor 70 delivers the straw to the hopper of a suitable press 71, preferably of the screw type to press out the black liquor contained therein, which black liquor may be conveyed by a suitable pipe 72 to the recovery system. In the first press the straw is still substantially in its stalk

structure, and by the action of the screw press the material is squeezed and mascerated, causing the extraction of heavy black liquor. In this pressing the stalk formations are distinegrated to a large degree.

From the press 71 the straw pulp is preferably saturated by wash water through suitable sprays 73 as it is carried along through a suitable conveyor, such as the helical conveyor 74, to a second screw press 75. The water for this purpose may be fresh water, or may be water from the pulp washing apparatus. Preferably, only as much wash water is added to the straw during its passage through the helical conveyor as the pulp will absorb without becoming liquid.

The weak black liquor extracted by the second press may be conveyed to the pipe 76 and sprays 45 to wash the cooked straw while in baskets, as mentioned above. If desired, however, it may be passed directly to the pipe 72, which leads to the black liquor recovery. A pipe 76a, together with valve 76b, is shown for this purpose as an optional connection.

From the second press the material is conveyed to a disintegrator in the form of a continuous breaker beater 78, in which water is added to reduce the pulp to a fluid condition. This beater has the usual perforated backfall 79, which operates as a screening and extraction device to prevent lumps of material passing through the machine. The roll is adjustable to the bed plate, so that controlled milling of unbroken stalk structures and the like may be effected along with the primary purpose of reducing the lumps of pulp delivered from the press to a uniform fluid condition.

From the breaker beater 78 the material goes through a suitable headbox 80 and is fed therefrom to a suitable refining engine, such as a Jordan refiner 81. While only one refiner is indicated in the drawings, it is to be understood that the pulp may be passed, if desired, through a plurality of refiners until it has been sufficiently refined.

The material coming from the refiner is sufficiently dilute so that it may be readily passed through a suitable screen 82, to which the material is carried by pipe 83. The purpose of the screen is to remove any nodes, weeds or stalks, etc., which have not been previously disintegrated. From the screen the material flows through headbox 84 to a washer 85, wherein the last remaining traces of cooking liquor are extracted. This washer may be one of a variety of forms, a suitable one being a multiple cylinder type washer commonly used in the paper industry, diagrammatically indicated at 85.

Such a washer may consist of any desired number of wire-cloth faced cylinders 86. For purposes of illustration a three cylinder washer is shown. In this washer the pulp is purified by addition of fresh water through pipe 87 at the final stage and, for economy of water, as well as with a view to recovery of some of the alkali in the wash water, a countercurrent system of connections is indicated, and the wash water emerging from the washer 85 passes to a waste tank 85a, from which it may be conducted by pump 85b through pipe 85c to the spray 73. An additional connection is shown by which the wash water may, if desired, be merged with the weak black liquor in pipe 76 from the second pressing operation. This connection comprises pipe 85d and valve 85e. From the washer the pulp is preferably delivered to a stock chest 88.

From the stock chest 88 the pulp may be run directly to paper machines, or, if it is desired to ship the pulp to some other plant or manufacturer, the pulp from the stock chest may be run through headbox 89 and then through a wet machine 90, in which the pulp is formed in layers on a drum and removed therefrom as sheets 91 of wet lap for baling and shipment.

In order to carry out the process economically, a recovery system is provided for the black liquor obtained from the process. The black liquor to be recovered may come from several stages of the process. The black liquor washed from the baskets of cooked straw and the black liquor extracted by the first pressing operation are usually conducted directly to the recovery system. A portion of the cooking liquor, either from the drainings from the baskets, discharged from the cooking tank, or the black liquor withdrawn from the cooking tank for regulation of the carbonate concentration of the cooking liquor, may go directly to the recovery system. The weak black liquor from the second pressing operation is preferably strengthened by utilizing it for washing the baskets of cooked straw, but, if desired, it may also be sent directly to the recovery system.

#### Recovery system

Such black liquors from the process are first passed through a screen filter 100 of well known type, comprising a revolving wire screen 101 which removes any residual pulp or coarse fibers that may be therein. From the filter the black liquor goes to the storage tank 102.

In order to economically effect the recovery of the constituents of the black liquor it must be concentrated, preferably in multiple effect steam evaporators, in order to concentrate the liquor most efficiently. As illustrated, the liquor goes through pipe 103 to evaporators 104 and 105 of a multiple effect system, it being understood that more evaporators may be utilized, if desirable. By using multiple effect evaporators, steam economy results and a supply of distilled water is obtained, which is desirable for the subsequent dialyzing operation.

The black liquor preferably is directed through the evaporators from the last effect toward the first effect. In the drawings, by way of example, is shown a double effect evaporator. The black liquor flows to the second effect through pipe 103, thence to the first effect through pipe 106, and from the first effect is pumped by pump 107 to the storage black liquor tank 108 for receiving concentrated black liquor.

The condensate from the multiple effect evaporators is pumped through pipe 109 to the condensate tank 110. From the concentrated black liquor storage tank 108 the liquor is passed to a battery of dialyzing cells 111 which separate the free alkali content from the lignin content by osmotic diffusion through suitable diaphragms, such as vegetable parchment. The free alkali is diffused through the diaphragm into the distilled water supplied from the condensate tank 110. The concentrated black liquor and the water condensate are passed through the dialyzing cells in countercurrent flow, i. e., the fresh water first extracts the alkali from the black liquor weakest in alkali.

The dialyzers are preferably the type in which a series of vegetable parchment diaphragms are disposed between plates and the water and black liquor pass through a multiplicity of passages

separated only by such diaphragms in counter-current flow, as above mentioned. They may be of the type shown in my copending application Serial No. 6,019, filed February 11, 1935.

The water or white liquor emerging from the dialyzer will have received by dialysis substantially all the free alkali content of the black liquor in the form of caustic soda and sodium carbonate. Preferably, the apparatus will be so adjusted and operated that the water flowing through the dialyzers will yield a liquor of about twice the desired strength of the cooking liquor, such, for example, as about 3 or 4% alkali content. The white liquor is conducted through pipe 112 to storage tank 113, from which it may, at periodic intervals, be conducted to any one of a series of causticizing tanks 114. In the causticizing tanks lime is added and the mixture agitated and boiled, which results in conversion of the sodium carbonate present in the white liquor into caustic soda and calcium carbonate sludge. The calcium carbonate is allowed to settle and the clear liquor taken off above the level of the precipitated sludge by pipe 115 to the cooking liquor storage tank 116.

In the drawings is shown an assembly of three causticizing tanks, so that the boiling operation, the settling operation, and the washing of the sludge, may be carried on in rotation in the three tanks.

After boiling the white liquor with a predetermined amount of lime and allowing the calcium carbonate sludge to settle, it is preferable to make an extraction of the alkali liquor from the sludge by adding a weak liquor obtained from a subsequent washing, agitating the sludge and the added liquor, and permitting the sludge again to settle. Such clarified weak liquor is then added to the first liquor to form the cooking liquor, and, if the white liquor coming from the dialyzer is of about double the strength desired for cooking, dilution with the clarified weak liquor just described renders the liquor of substantially the proper strength for cooking additional fibrous material.

It is usually economical to make a second extraction of alkali from the sludge, and, if it be desired to do this, fresh water is added and the mixture agitated and allowed to settle. This second weak liquor may be used in the previously described second extraction of lignins and solid material from the cooked fibrous material.

A collecting box 117 for collecting the water from the condenser 118 is provided, and such water may be supplied to the causticizing tanks. To this end a pump 119 and pipe 120 are shown. The supplying of the warm water from the condenser to the tanks is economical, since by its use the consumption of steam in causticizing is lessened. Also, this water may contain a slight amount of alkali which has been entrained in the vapor passing from the last effect of the evaporator to the condenser, and, by utilizing the condenser tail water in the causticizing tank, such alkali as may be present in this water is conserved for use in the process.

The liquor containing lignins emerging from the dialyzers passes through pipe 121 to the lignin evaporator 122, where it is further evaporated, preferably by steam from steam pipe 123. The lignins are carried from the evaporator by pump 124 and pipe 125, where the liquid lignins may be put in barrels 126 for shipment. A portion or all of the liquid lignins may, if desired, be passed to the film evaporator, which comprises a tank 127

and heated drum 128, from which the dried film may be removed and passed to a suitable conveyor 129 for taking the dried material to a suitable place for storage or shipment. The lignins produced by this process have commercial utility. They may be used as binders in various compositions, or certain of the constituent parts may be segregated for use in various arts and industries.

It will be seen that according to the method and apparatus disclosed in this application, which is a continuation-in-part of my application Serial No. 6,019, filed February 11, 1935, for Pulp production process and apparatus, a simple and flexible control of the cooking of straw and the like is readily obtained. By withdrawing cooking liquor from the outlet portion of the tank, either continuously or intermittently, reheating, and returning a portion of the liquor to the tank, the temperature of the cooking liquor may be maintained substantially constant, the causticity and sodium carbonate concentration may be readily maintained within predetermined desirable limits, and, of course, the time of cooking is entirely within the control of the operator as the unit containers of straw may be passed through the cooking tank at any desired speed.

By cooking at temperatures below the boiling point, stronger fiber is obtained than when cooking under pressure at high temperatures, and, also, disintegration of the nodes and other matter deleterious to the quality of the pulp is minimized. The maintenance of the strength of the caustic alkali substantially constant, or within predetermined limits, is also very advantageous.

With the recovery system provided it is possible to use an excess of alkali in the cooking bath over that actually needed for chemical combination with the ligneous material, and, accordingly, the chemical action may be effected at temperatures lower than could be used in systems employing quantities of chemical and raw material proportioned to achieve practically a complete exhaustion of the alkali at the completion of the cook, as, for example, in batch cooking in pressure digesters.

The time of cooking is reduced and the efficiency of the cooking is increased by utilizing the countercurrent flow principle, that is, in adding fresh cooking liquor at the end of the tank where the cooking of the straw is substantially completed.

It may also be noted that maceration and mechanical action on the straw is avoided during cooking and subsequent draining of the cooking liquor from the straw in the containers, so that a much higher recovery of cooking liquor by drainage results, as the liquor will drain more readily from the unbroken stalks than it will from a quantity of macerated fiber. Also, the preliminary washing of the straw is provided for in my apparatus prior to the mechanical action on the straw, which further facilitates the high recovery of cooking liquor.

By making provision for thoroughly wetting, wilting and compacting the straw before charging it into the cooking containers the capacity of the containers is greatly increased and the productive capacity of the cooking tank is increased.

The provision of means for successively squeezing, wetting, and again squeezing the cooked straw previous to the final washing aids the extraction of the cooking liquor not previously removed from the straw. The liquor obtained by the first squeezing operation may pass directly to the black liquor recovery system, and preferably

the liquor obtained from the second squeezing may be utilized, as indicated above, to extract further cooking liquor from the straw while it is still in the cooking container, and then may be sent through the recovery system.

The provision of means for separation of the ligneous soaps from the free alkali content of the black liquor permits recovery of both the caustic soda and sodium carbonate which may be present in the liquor, and the solution may be recausticized with lime for repeated use in the process of cooking straw. The lignins, after extraction by dialysis of the free alkali content from the black liquor, may be saved and used industrially for many purposes. This saving of the lignins is a distinct advantage of the process, in that it has been customary to incinerate or calcine the black liquors to recover the sodium content, and this method involved a total loss of the ligneous material.

By the process of dialysis for separation of the free alkali content from the ligneous matter in the black liquor, such caustic soda as exists as such in the black liquor is not first converted into sodium carbonate prior to recausticizing, as is the case in the recovery process in which the black liquor is incinerated or calcined. Thus, less lime is required for recausticizing the sodium carbonate and economies are effected in recovering the caustic soda for reuse in cooking.

Furthermore, it is to be understood that the particular forms of apparatus shown and described, and the particular procedure set forth, are presented for purposes of explanation and illustration, and that various modifications of said apparatus and procedure can be made without departing from my invention, as defined in the appended claims.

What I claim is:

1. In the preparation of pulp from straw, the method of continuously cutting, wilting and compacting the straw, loading the compacted straw into successive foraminous containers, substantially submerging said containers in a mild, hot sodium hydroxide liquor and passing them through the cooking liquor at a predetermined rate at substantially atmospheric pressure and at a temperature below the boiling point of such liquor, withdrawing the container from the cooking liquor, and returning the cooking liquor that drains from said containers to the cooking liquor tank.

2. In the preparation of paper forming stock from straw, the method which comprises submerging the straw in unit containers in a mild alkaline cooking liquor at a temperature below the boiling point and at substantially atmospheric pressure, and controlling the cooking by maintaining the causticity of the cooking liquor and regulating the concentration of the sodium carbonate within the cooking liquor within predetermined limits.

3. In the preparation of paper forming stock from straw, the method which comprises submerging the straw in unit containers in a mild alkaline cooking liquor at a temperature below the boiling point and at substantially atmospheric pressure, and controlling the cooking by maintaining the proportions of sodium hydroxide

and carbonates within the desired limits in the cooking liquor.

4. In the preparation of paper forming stock from straw, the method which comprises submerging the straw in unit containers in a mild alkaline cooking liquor at a temperature below the boiling point and at substantially atmospheric pressure, and controlling the cooking by regulating the causticity of the cooking liquor and maintaining the lignin concentration within predetermined limits.

5. In combination, a cooking tank adapted to contain a hot, alkaline cooking liquor, means for introducing and submerging in the cooking liquor foraminous unit containers loaded with wet, compacted straw, means for passing the containers through the cooking liquor at a predetermined rate, a drainage runway for the containers, means for withdrawing the unit containers from the cooking liquor and placing them on said runway, means for delivering the liquor drained from said containers into the tank, and means for maintaining the temperature and causticity of the cooking liquor substantially constant.

6. In combination, a cooking tank adapted to contain a hot, alkaline cooking liquor, means for introducing and submerging in the cooking liquor foraminous unit containers loaded with wet, compacted straw, means for passing the containers through the liquor and causing countercurrent relative movement of the containers and liquor, a drainage runway for the containers, means for withdrawing the unit containers from the cooking liquor and placing them on said runway, means for delivering the liquor drained from said containers into the tank, and means for maintaining the temperature and causticity of the cooking liquor substantially constant.

7. In the preparation of pulp from straw, the steps which comprise submerging the straw in a hot, dilute, alkaline liquor, withdrawing portions of the liquor from time to time as it becomes charged with organic material extracted from the straw, concentrating the withdrawn liquor in steam heated evaporators and conserving the steam condensate obtained from the evaporation, causing a countercurrent flow of the concentrated black liquor and warm condensate in alternate dialytic cells separated by vegetable parchment membranes, whereby the uncombined alkali content of the black liquor is recovered for cooking additional straw and a ligneous product is conserved.

8. In the preparation of pulp from straw and the like, the method which comprises introducing unit carriers containing wilted, cut straw into a bath of mild, hot, alkaline cooking liquor of a strength below 5% at substantially atmospheric pressure for a predetermined time, removing the units of cooked straw from the bath and permitting the cooking liquor to drain from the cooked straw into the cooking bath, removing the straw from the containers, extracting the remaining black liquor in the straw and macerating the straw, and subjecting the straw to a mechanical defibering treatment to reduce it to pulp.

MAX SKOLNIK.